

Aug. 27, 1957

W. J. WALLACE

2,804,407

PROCESS FOR DESCALING TITANIUM

Filed Sept. 6, 1955



INVENTOR.

W. J. WALLACE

BY

S. T. Tamm Jr.  
ATTORNEY

## 1

2,804,407

## PROCESS FOR DESCALING TITANIUM

Wilfred J. Wallace, Chula Vista, Calif., assignor to Rohr Aircraft Corporation, Chula Vista, Calif., a corporation of California

Application September 6, 1955, Serial No. 532,538

6 Claims. (Cl. 148—6.14)

This invention relates to a process for treating metal parts made of titanium which have to be heated to form the parts to a desired shape or for other purpose and during which treatment oxides are formed on the parts which are normally very difficult to remove. It is believed that the oxide film usually formed when the uncoated metal is heated to from 400° to 1400° F. consists largely of the higher oxides of the metal such as  $TiO_2$  and  $TiO_3$  and that such oxides are difficult to later remove.

Furthermore oxidation in the presence of air proceeds rapidly at high temperatures so that a rather thick layer of oxides is formed thereby detracting from the strength of the part. This impairment of strength is especially marked when the parts are formed of thin sheet titanium having a thickness from .012 to .050 inch.

It is an object of this invention to provide a treatment for one or more titanium parts which require heat treatment which assures the formation of thin film of oxide or oxides of titanium on the surface of the metal, during the heating, which film can later be completely and easily removed.

Another object is to provide a treatment for a titanium part or parts which require heat treatment up to a temperature of from 900° to 1400° F. which forms a thin protecting film on the parts consisting of the lower oxides of titanium, this film being formed while the temperature of the parts is increasing within the range of approximately 400° to 500° F. and protecting the metal from further oxidation as the temperature of the parts continues to increase.

A further object is to provide a treatment which will quickly and completely remove the scale formed during the heating operation and leave the exposed surface of the finished part clean and free from scale.

Further objects will become apparent as the description of the treatment proceeds. For a better understanding of the invention reference is made to the accompanying drawing, in which:

Fig. 1 is a sectional view of a tank containing a titanium sheet immersed in a treating liquid in the tank;

Fig. 2 is a diagrammatic sectional view of a heating furnace;

Fig. 3 is a diagrammatic view, partly in section of a forming press used in the process and;

Fig. 4 is a sectional view of a tank containing a treated sheet immersed in a descaling bath.

The sheet 10 of titanium to be treated is first dipped in a bath 11 contained in a tank 12 made of material which is not affected by the chemicals in the bath. The bath is preferably kept at a temperature of from 75 to 80° F. by any suitable heating means as, for example, a steam pipe 13 passing through the tank.

The bath is made by heating water to the temperature named, adding sodium or potassium nitrate and sodium or potassium carbonate and stirring or agitating till the salts are dissolved. Sodium aryl sulfonate is then added and the bath again stirred. Next isopropyl or isobutyl

## 2

alcohol is added and the bath slightly agitated. These materials are added in suitable amounts to provide an aqueous solution of the following proportions by weight:

|                               | Percent    |
|-------------------------------|------------|
| 5 Sodium or potassium nitrate | About 40   |
| Sodium or potassium carbonate | 2 to 3     |
| Alcohol                       | 0.8 to 4.0 |
| Sodium aryl sulfonate         | About 0.01 |
| Water                         | Balance    |

Instead of the alcohols mentioned any of the alcohols completely soluble in water and having a vapor pressure of from 40 to 80 millimeters of mercury at 20° C. may be used instead. The sulfonate acts as a wetting agent by reducing the surface tension of the solution and facilitating the complete wetting of the sheet.

After the sheet is wet, it is removed from the bath and allowed to dry in a current of slowly moving air at a temperature from 70 to 180° F. The alcohol evaporates and assists the wet coating on the sheet to dry rapidly. The sheet is now coated with a thin film of material which will cause titanium oxides of desired composition to form when the sheet is heated to form it to a desired shape.

25 *Heating*

The dry coated sheet or sheets are now heated to the required forming temperature in a furnace 14 which is opened by a door 15 sliding in guides 16. The interior of the furnace is heated to the required forming temperature usually within the range of 400 to 1200° F. depending on the extent to which the sheet has to be bent to conform it to the desired shape by the forming die. This heating may be done by any suitable means such as electric heaters 17 embedded in the floor or wall of the furnace.

As the heating proceeds and the sheet passes from 400° to 500° F., oxygen is liberated from the alkali nitrate, this oxygen uniting with the titanium to form a thin film composed essentially of the lower oxides of the metal, believed to be  $Ti_2O_3$ ,  $Ti_3O_4$  or a mixture of both oxides. The carbonate present lowers the fusion point of the mixture on the metal and also has a reducing action which limits the formation of higher oxides such as the dioxide  $TiO_2$  and trioxide  $TiO_3$  whose presence is undesirable and would make complete removal of the scale from the articles more difficult. As the sulfonate present is heated above 300° F. it decomposes and has a reducing action which tends to prevent the formation of the higher oxides of the metal.

50 If it is necessary to increase the temperature beyond 500° F., the film of the lower oxides of titanium which have been formed on the surface of the sheet acts as a barrier to prevent the oxidation from penetrating further into the metal and also prevents formation of the deleterious higher oxides such as  $TiO_2$  and  $TiO_3$ .

55 *Forming*

When the sheet has reached the required forming temperature, the door 15 of the furnace is raised, the coated sheet removed from the furnace and the hot sheet immediately put on female forming die 18. This die is supported on a fixed anvil 19 and may be at room temperature. When a deep draw is required however, the die is preferably heated, as by electric heating coils 20 embedded in the die, to a temperature of from 400 to 800° F. The male die 21 is immediately lowered to press the sheet against die 18 and form it to the desired shape. Die 21 is shown as mounted on a ram 22 which is connected to a piston rod 23 operated by a piston 24 slideable in cylinder 25. Compressed air is admitted in a known manner above the piston from a pipe 26 or below the piston from pipe 27. The usual vertical guides (not shown)

cooperate with ram 22 to prevent it from turning. After forming, compressed air is admitted to pipe 27 which raises the die 21 when the formed sheet is removed and allowed to cool to room temperature (about 70° F.). The formed sheet is now ready for having the adherent scale removed from its surface.

#### Descaling

The removal of the scale is effected by immersing the formed sheet 10 in an acidic bath 28 contained in a tank 29 which is lined with a plastic which bath 28 will not attack. The bath is preferably kept at a temperature of from 110° to 130° F. by any suitable heating means such as steam passing through a pipe or coil 30 which passes through the tank and bath. Normally the scale is completely dissolved in from 30 to 60 seconds but a somewhat longer immersion may be needed in some cases to completely remove the scale. Bath 28 is preferably an aqueous solution of the following proportions by weight:

|                                               | Percent  |
|-----------------------------------------------|----------|
| Nitric acid                                   | About 29 |
| Ammonium bifluoride, $\text{NH}_4\text{HF}_2$ | About 2  |
| Water                                         | Balance  |

Instead of the ammonium bifluoride an equal weight of sodium fluoride may be used instead or about 2.5 percent of technical grade 60 percent hydrofluoric acid (HF) may be mixed with the nitric acid solution.

Upon removal from bath 28, the sheet is rinsed in water to remove the descale solution and allowed to dry. The surface of the finished sheet is of uniform color and free from scale which would detract from its appearance.

An alternative method for securing clean formed sheets of good appearance is to first heat the sheet without any previous treatment in furnace 14 to the forming temperature (600° to 1400° F.). This heating produces an oxide film or coating of the higher oxides of titanium  $\text{TiO}_2$  and/or  $\text{Ti}_2\text{O}_3$  on the sheet. The coated sheet while hot is placed on die 18 and formed in the manner above described. The sheet is then allowed to cool and any grease or other lubricant which was used on it to facilitate the forming is removed in a known manner. The oxide coated sheet is then dipped in bath 11 of the composition above described, removed from the bath and allowed to dry. The formed sheet is now placed in furnace 14 and reheated to the forming temperature. This reheat causes the chemicals on the oxide film to reduce the higher oxides therein to the lower oxides ( $\text{TiO}_2$  and/or  $\text{Ti}_2\text{O}_3$ ) and also relieves the sheet of any internal stresses which may have been set up therein by the forming. The sheet is now removed from the furnace, placed on die 18 again and pressed lightly by die 21 again to remove any distortion which the reheating may have caused.

The scale remaining on the sheet is now removed by the descaling process above described whereupon the formed sheet is ready for sale or for assembly with other parts into a composite structure.

While the above description has referred to the treatment of a single sheet, it will be understood that a number of sheets may be treated in baths 11 and 28 simultaneously and also that a number of sheets may be heated in furnace 14 simultaneously.

This invention may be embodied in other forms or carried out in other ways without departing from the spirit or essential characteristics thereof. The present embodiment of the invention is therefore to be considered as in all respects illustrative and not restrictive, the scope of the invention being indicated by the appended claims, and all changes which come within the meaning and range of equivalency of the claims are intended to be embraced therein.

Having thus described my invention, what I claim as new and useful and desire to secure by Letters Patent is:

1. The method of forming a sheet of titanium to the

shape of a curved die which comprises the steps of dissolving a salt of the group consisting of sodium nitrate and potassium nitrate and a salt of the group consisting of sodium carbonate and potassium carbonate in water; heating the aqueous solution to a temperature within the range of 75° to 80° F.; dipping the entire sheet in the heated solution; drying the wet sheet to leave a thin oxygen-containing coating thereon; heating the coated sheet in the presence of air to a temperature within the range of 400 to 1200° F. to oxidize the surface thereof; and pressing the hot oxidized sheet against said die.

2. The method of treating a formed sheet of titanium which has previously been heated to a high temperature and is coated with a surface film composed of the higher oxides of titanium, which comprises the steps of dipping the entire sheet in an aqueous solution of a salt of the group consisting of sodium nitrate and potassium nitrate and a salt of the group consisting of sodium carbonate and potassium carbonate; drying the wet coated sheet; and heating the dry coated sheet to a temperature higher than 400° F. to reduce the higher oxides of titanium in the surface film.

3. The method of forming a titanium sheet to the contour of a curved die which comprises the steps of treating the sheet with a salt solution at a temperature about 75° F., said solution consisting essentially of a salt of the group consisting of sodium nitrate and potassium nitrate, a salt of the group consisting of sodium carbonate and potassium carbonate, and water; drying the wet sheet to leave a thin oxygen-containing coating thereon; heating the coated sheet to a temperature above 400° F. to soften the sheet for forming and oxidizing the surface thereof; pressing the heated sheet against the face of the die; removing the heated sheet from the die; and treating the formed sheet with an aqueous solution of nitric acid and ammonium bifluoride to dissolve the scale on the sheet.

4. The method of forming a thin sheet of titanium to the shape of a curved die face which comprises the steps of wetting the entire sheet with an aqueous solution consisting essentially of sodium nitrate about 40 percent, sodium carbonate about 2 to 3 percent, balance water; drying the wetted sheet to provide a thin dry surface film thereon; heating the treated sheet to a temperature within the range of 400° to 1200° F. to provide a thin surface coating of the lower oxides of titanium thereon; and pressing the hot coated sheet against said die face.

5. The method forming a thin sheet of titanium to the shape of a curved die face which comprises the steps of wetting the entire sheet with an aqueous solution consisting essentially of potassium nitrate about 40 percent, potassium carbonate about 2 to 3 percent, balance water; drying the wetted sheet to provide a thin dry surface film thereon; heating the treated sheet to a temperature within the range of 400° to 1200° F. to provide a thin surface coating of the lower oxides of titanium thereon; and pressing the hot coated sheet against said die face.

6. The method of forming a sheet of titanium to the shape of a curved die which comprises the steps of dissolving a salt of the group consisting of sodium nitrate and potassium nitrate and a salt of the group consisting of sodium carbonate and potassium carbonate in water to provide a bath; adding about 1 percent of alcohol whose vapor pressure is between 40 and 80 millimeters of mercury at 20° C. and about 0.01 percent of a soluble surface tension-reducing compound to the bath; dipping the entire sheet in the bath; drying the wet sheet to leave a thin oxygen-containing coating thereon; heating the coated sheet in the presence of air to a temperature within the range of 400° to 1200° F. to oxidize the surface of the sheet; and pressing the hot treated sheet against said die.

References Cited in the file of this patent

UNITED STATES PATENTS

2,289,443 Monge July 14, 1942

(Other references on following page)

5

## UNITED STATES PATENTS

2,309,745 Bergin ----- Feb. 2, 1943  
2,499,764 Mabus ----- Mar. 7, 1950  
2,554,042 Mayfield ----- May 22, 1951  
2,598,889 Caugherty ----- June 3, 1952  
2,704,883 Hamilton et al. ----- Mar. 29, 1955  
2,724,667 McPherson ----- Nov. 22, 1955

6

## FOREIGN PATENTS

734,859 Germany ----- Apr. 29, 1943  
OTHER REFERENCES

5 Handbook on Titanium by Adenstedt, August 1954,  
pages 1-3-15.